

# UNITED STATES PATENT OFFICE.

FRANK D. BELKNAP, OF NEW YORK, N. Y.

## STENCIL-SHEET.

1,101,241.

Specification of Letters Patent. Patented June 23, 1914.

No Drawing.

Application filed May 4, 1912. Serial No. 495,309.

*To all whom it may concern:*

Be it known that I, FRANK D. BELKNAP, a citizen of the United States of America, residing at New York city, borough of Manhattan, county and State of New York, have invented certain new and useful Improvements in Stencil-Sheets, of which the following is a specification.

My invention comprises an improved 10 stencil and the sheet from which said stencil may be made by the operation of an ordinary typewriting machine or similar apparatus. Stencils have been heretofore produced by treating loose fibered papers with 15 various compositions but all of these have been subject to serious disadvantages. Paper treated with wax or paraffin is liable to injury by wrinkling, bending or breaking, the ink in the after operation penetrating 20 the paper along the lines of breakage, thus producing inferior or useless results. In addition to this disadvantage, it has been found that they are not capable of a sufficient number of repeated uses and that they 25 deteriorate very badly with age. Attempts have been made to use other compositions which would avoid these particular defects, but the sheets thus produced require to be moistened before the stencil impressions can 30 be properly formed therein.

The primary object of my invention is to produce a sheet capable of being stencilized, formed by treating a sheet of loose fibered material such as Yoshino paper, with a suitable 35 substance, or combination of substances, so that the stencil characters may be formed without previous dampening of the sheet and which will not be damaged by wrinkling, bending or breaking, as is the case 40 with papers now upon the market.

The resultant product of my invention forms a most efficient stencil blank which can be stencilized in an ordinary typewriting machine without remoistening and without 45 injury by ordinary handling or injury to typewriter by water. The stencil sheets so formed can be used to produce an indefinite number of copies, either by hand or in any suitable machine, and will not appreciably 50 deteriorate from age, usage, or ordinary handling.

When a sheet of paper treated with my improved process is operated on by an ordinary typewriter or equivalent apparatus, the 55 material incasing and permeating the fibers of the paper is forced aside wherever the

type strikes the sheet, thus leaving the loose fibers of the paper practically bare at those points. When ink is applied to one side of the sheet it passes through these exposed 60 surfaces of fiber and the characters which have been impressed on the stencil sheet are thus inked on a sheet of paper or other surface placed beneath, the resulting characters closely reproducing those which would have 65 been printed thereon if the sheet of paper had been used in the typewriter in the usual way.

Broadly stated, my invention comprises the saturation of a sheet of loose fibered 70 material, for instance Yoshino paper, with a gelatinous material, such as commercial gelatin, Irish moss, vegetable gum, either alone or in mixtures with each other, a salt of fatty acid, such as soap and a hygroscopic 75 substance, such as glycerin. Preferably, an oxidizing agent, such as hydrogen peroxid, is also employed as a purifier and coagulant.

In carrying out my invention in its best form, as at present known to me, I take, one 80 ounce of castile soap (or the equivalent amount of ingredients of said soap, *i. e.*, olive oil and caustic soda), 2 ounces of glycerin, 4 ounces of animal gelatin, (or 2 ounces of gelatin and 2 ounces of Irish 85 moss), and about 120 ounces of water. This mixture is thoroughly dissolved and mixed under the influence of heat. On the surface of this solution, preferably warm, is laid a sheet of Yoshino paper, which immediately 90 absorbs the necessary quantity of the solution. In removing the sheet, it is advisable to draw it over sharp, straight edges of metal to insure a uniform distribution of the material on its surface. After the sheet 95 has been dried by exposure to the atmosphere or otherwise, it is subjected to a second bath, preferably, at the room temperature, composed of 1 ounce of hydrogen peroxid and 2 ounces of glycerin, dissolved 100 in about 6 ounces of water, and the sheet is again allowed to dry. So far as I am at present advised the principal functions of the soap included in the foregoing formula are to act as a softening agent and also to 105 increase the imperviousness of the film formed on the paper. It seems to heighten the imperviousness of the film by acting as an ink repellent, preventing the ink being sucked by capillary action through occasional pores of the treated sheet. I believe 110 that the soap also has a minor beneficial ac-

tion in holding the glycerin more firmly fixed in the solution, and in the coating produced thereby.

In following the above operation, I do not limit myself to the proportions, the identical ingredients, or the temperatures cited, all of which may be varied without departing from the essence of my invention. The two operations, as above mentioned, may be combined into one, by adding the hydrogen peroxid and the last addition of glycerin to the first bath, but under these conditions it is advisable that the temperature of the bath should be somewhat lower than has been found advisable where the second bath operation is employed. Certain of the ingredients above specified can be omitted without departing from my invention and without destroying the usefulness of the product, but the best results that I have thus far obtained are produced by following the procedure above outlined.

Claims.

1. A stencil sheet formed of a base of loose fibered paper treated with solutions comprising glycerin, a gelatinous material, castile soap and hydrogen peroxid.
2. A stencil sheet formed of a base of loose fibered material saturated with an aqueous solution comprising a gelatinous material, glycerin and a vegetable soap.
3. A blank capable of being stencilized comprising a loose fibered paper as a base and a coating comprising a gelatinous material, glycerin, castile soap and hydrogen peroxid.
4. A blank capable of being stencilized comprising a loose fibered paper as a base and a coating comprising a gelatinous material, glycerin, and a vegetable soap.
5. A blank capable of being stencilized comprising a base of Yoshino paper, saturated with a composition comprising gelatin, glycerin, a vegetable oil, a caustic alkali, and hydrogen peroxid.
6. A blank capable of being stencilized comprising a sheet of loose fibered material treated with animal gelatin, Irish moss, glycerin and a salt of a fatty acid.
7. A blank capable of being stencilized comprising a sheet of loose fibered material treated with animal gelatin, Irish moss, glycerin, a salt of a fatty acid and an oxidizing agent.
8. A blank capable of being stencilized comprising a sheet of loose fibered material treated with a gelatinous material, a salt of a fatty acid, and a hygroscopic substance.
9. A blank capable of being stencilized,

comprising a sheet of loose fibered material treated with a gelatinous material, a salt of a fatty acid, and glycerin.

10. A blank capable of being stencilized, comprising a sheet of loose fibered material treated with a gelatinous material, an alkali salt of a fatty acid, and a hygroscopic substance.

11. A blank capable of being stencilized, comprising a sheet of loose fibered material treated with a gelatinous material, an alkali salt of a fatty acid, and glycerin.

12. A blank capable of being stencilized, comprising a sheet of loose fibered material treated with a gelatinous material, a saponified fat, and a hygroscopic substance.

13. A blank capable of being stencilized, comprising a sheet of loose fibered material treated with a gelatinous material, saponified olive oil, and glycerin.

14. A blank capable of being stencilized, comprising a sheet of loose fibered material treated with a gelatinous material, a salt of a fatty acid, a hygroscopic substance, and an oxidizing agent.

15. A blank capable of being stencilized, comprising a sheet of loose fibered material, treated with a gelatinous material, a salt of a fatty acid, glycerin, and an oxidizing agent.

16. A blank capable of being stencilized, comprising a sheet of loose fibered material treated with a gelatinous material, a salt of a fatty acid, glycerin, and hydrogen peroxid.

17. A blank capable of being stencilized, comprising a sheet of loose fibered material treated with a gelatinous material, an alkali salt of a fatty acid, glycerin, and hydrogen peroxid.

18. A blank capable of being stencilized, comprising a sheet of loose fibered material treated with a gelatinous material, saponified olive oil, glycerin, and hydrogen peroxid.

19. A blank capable of being stencilized, comprising a sheet of loose fibered material treated with a gelatinous material, an alkali salt of a fatty acid, a hygroscopic substance and an oxidizing agent.

20. A sheet capable of being stencilized by printing type without the external application of moisture, comprising a thin, loose fibered sheet of paper treated with gelatin, glycerin, Irish moss and a coagulant.

FRANK D. BELKNAP.

Witnesses:

SAMUEL WEINBERG,  
MAI FILES.